

G. H. Smith.  
Iron & Steel Direct.  
No 91,894. Patented Jul 20, 1869.



Witnesses:  
Andrew De Lacy  
W. H. Bishop

Inventor:  
George Hand Smith

# United States Patent Office.

GEORGE HAND SMITH, OF NEW YORK, N. Y.

Letters Patent No. 92,894, dated July 20, 1869.

## IMPROVEMENT IN THE MANUFACTURE OF WROUGHT-IRON AND STEEL DIRECT FROM THE ORE.

The Schedule referred to in these Letters Patent and making part of the same.

To all whom it may concern:

Be it known that I, GEORGE HAND SMITH, of the city, county, and State of New York, have invented a new and useful Improvement in the Process of Making Wrought-Iron and Steel Direct from the Ore; and I do hereby declare that the following is a full, clear, and exact description thereof, reference being had to the accompanying drawings, making part of this specification, illustrative of a furnace suitable for, and which may be used in working my said improved process, in which drawings—

Figure 1 is a longitudinal vertical section.

The other figure will be referred to hereafter.

The object of my invention is to obtain wrought-iron or steel directly from iron-ore, without fusion of the ore, so that wrought iron or steel of uniform grades can be obtained at less cost than by any other known process; and, to that end,

My said process consists in heating the ore, after it has been mechanically reduced, by neutral heat, in a suitable furnace, until it reaches a white heat, short of fusion of the ore, and then introducing into the charge so heated, and from a separate source, carbonaceous gas or vapor, to effect the conversion of the ore into wrought-iron or steel, suitable for balling up and working into blooms and finished bars, or for melting to produce cast-steel.

For the working of my said process, I take the ore, by preference the rich black oxides and specular varieties, and, by any of the well-known or suitable means, reduce it mechanically to small lumps, by preference so that the largest will pass through a screen of three-quarter-inch meshes.

So reduced, the ore is charged, to the depth of from six to eight inches, on the floor *a* of either of the furnaces represented in the accompanying drawings.

The furnace for the working of my said process must have at least three compartments, viz:

First, a converting-chamber, *a*, on the floor of which the comminuted ore is charged, to the depth of from six to eight inches.

Second, a fire-chamber, *b*, for the charge of heating-fuel, provided with a suitable grate and means for introducing a blast of air, and so located that the flame and gaseous products of the combustion will pass over the charge of ore, and return in a flue, *c*, under the floor of the converting-chamber.

Third, a chamber, *d*, for containing the charge of carbonaceous matter, which chamber must be separate from the fire-chamber and from the converting-chamber, but in such proximity to the converting-chamber that the carbonaceous gases generated may be readily transferred to the converting-chamber, to act on the heated ore.

I prefer to locate the third chamber, *d*, for containing the carbonaceous matter, immediately between the

first or converting-chamber and the second or fire-chamber, so that the roof of the third chamber shall constitute the bridge of the fire-chamber, that the carbonaceous matter may be thereby heated.

The furnace may be double, as in Figure 2, the two converting-chambers being separated by a wall, *e*.

In working my said process, I so manage the fire in the fire-chamber as to obtain neutral heat, by which I mean that no oxygen, or but very little, shall escape from the fire-chamber into the converting-chamber, which is effected by a deep charge of fuel, compared with the blast of air, that all the oxygen of the air may be taken up by the carbon of the fuel.

The object is so to regulate the supply of fuel and the blast of air, that the gases evolved from the fire-chamber will be, as near as can be, carbonic acid, containing neither oxygen nor carbon in a condition to act upon the ore. The manner in which such a fire is to be managed will be readily understood by experienced iron-masters.

The third or carbon-chamber is separated from the converting-chamber by a bridge, *f*, there being sufficient space between the said bridge and the roof *g* for the passage of the carbonaceous vapor into the converting-chamber, to act upon the heated ore.

After the ore has been heated up to a white heat, a little short of a welding-heat, the carbonaceous matter is introduced into the carbon-chamber, through a suitable aperture, and there vaporized, that in the gaseous form it may escape to act upon and convert the ore.

The carbonaceous matter may be bituminous coal, or any of the hydrocarbons, or other volatile carbonaceous matter, but other carbonaceous matter, such as coke or charcoal, may be substituted, if ignited in the chamber and supplied with atmospheric air in such proportion as to produce carbonic oxide.

During the time that the carbonaceous gases are being introduced, the ore should be occasionally stirred and turned over, through apertures in the side walls, that every part of the charge may be converted, which will take from two to six hours, depending upon the depth of the charge and the size to which the ore has been granulated, and the extent to which it may be desired to apply carbon.

The required degree of conversion is determined by taking portions of the ore out of the furnace and subjecting them to the required tests.

The ore, when ascertained to be properly converted, is taken out of the furnace, and transferred to any suitable balling-furnace, where it is balled, and then hammered or rolled. But if desired, instead of balling the converted ore, it may be melted in crucibles or suitable furnaces, and made into either cast-steel or wrought-iron.

It will be seen, that when the said process is used

for making wrought-iron, the application of the carbonaceous vapor is stopped so soon as the heated ore is deoxidized; and when making steel, it is continued beyond the deoxidization of the heated ore, until the required degree of carbonization has been obtained, depending upon the grade of steel desired.

I do not wish to be understood as limiting myself to the working of my said process in a furnace such as I have herein described, as it may be worked in furnaces of different construction. The furnace represented in the accompanying drawings will be found suitable for the purpose.

Various processes have been described and tried for making wrought-iron and steel directly from the ore, all of which have been found to be more or less defective, uncertain in the results, and too expensive. I do

not, therefore, wish to be understood as making claim, broadly, to the making of wrought-iron and steel directly from the ore; but

What I do claim as my invention, and desire to secure by Letters Patent, is—

Heating the ore to a white heat, by what I have herein described as neutral heat, and while the ore is in that state, applying to it the required charge of carbon, in the gaseous form, from a source separate from the heating-fire, to effect the conversion of the ore, substantially as and for the purpose specified.

GEORGE HAND SMITH.

Witnesses:

Wm. H. BISHOP,  
ANDREW DE LACY.